

## UNITED STATES PATENT OFFICE.

ARTHUR HOUGH, OF SUMMIT, NEW JERSEY.

## TREATMENT OF VEGETABLE PARCHMENT.

No Drawing.

Application filed April 23, 1923. Serial No. 634,181.

*To all whom it may concern:*

Be it known that ARTHUR HOUGH, a citizen of the United States of America, residing at Summit, in the county of Union and State 5 of New Jersey, has invented certain new and useful Improvements in the Treatment of Vegetable Parchment, of which the following is a specification.

The present invention relates to improvements in the preparation of parchment paper which is commonly referred to as vegetable parchment.

As is well known, vegetable parchment is prepared by treating paper with sulfuric acid of a proper strength, and subsequently washing to remove the acid, after which the parchment is dried. After drying the vegetable parchment is somewhat brittle, and if not brittle when first made, it is likely to 20 become brittle on long storage, particularly in very dry rooms.

I have found that it is possible to keep vegetable parchment permanently soft, by coating the same with a small quantity of a glycol. For ordinary purposes I prefer to use ethylene glycol, this being a dihydric alcohol which is already well known and which is described in numerous text books of organic chemistry. This material has 30 properties which render it especially suitable for use, in the form of a thin coating, on vegetable parchment. It has a favorable degree of viscosity, can readily be prepared in a very pure condition, and it possesses no 35 injurious effects upon the human system, which latter properties render it particularly desirable, when the parchment paper is to be used for wrapping food products.

For ordinary purposes I find that the application of approximately 200 pounds of ethylene glycol to each ton of paper gives 40 very satisfactory results, the same being applied as a particularly uniform coating over one or both sides of the parchment. The parchment can then be rolled up in the form of rolls or stored in the form of sheets, and does not become brittle by the excessive drying out. It will be understood that in place 45 of the simple glycol, its polymers would likewise be employed, for instance diethylene glycol, the term "ethylene glycol" as used in this application is intended to cover the polymers as well. The glycol is somewhat 50 hygroscopic and takes up a certain amount of moisture from the atmosphere, retaining 55 the necessary quantity of moisture in the paper at all times to prevent the paper from becoming brittle owing to excessive drying out.

I claim:

1. The herein described process which comprises applying a glycol to paper material.
2. A process which comprises applying a coating of ethylene glycol to parchmentized 65 paper, whereby the paper is kept soft and pliable for a long period.

In testimony whereof I affix my signature in presence of two witnesses.

ARTHUR HOUGH.

Witnesses:

J. F. WELLER,  
EUGENE JOB.